

# United States Patent Office

3,291,609

Patented Dec. 13, 1966

1

3,291,609

## DEVELOPER INCORPORATED PHOTOGRAPHIC MATERIALS

Ralph Frederick Porter, Pittsford, and Thomas Edward Gompf, Penfield, N.Y., assignors to Eastman Kodak Company, Rochester, N.Y., a corporation of New Jersey

No Drawing. Filed June 5, 1964, Ser. No. 373,050

11 Claims. (Cl. 96—76)

This application is a continuation-in-part of our pending application Serial No. 183,354, filed March 29, 1962, now abandoned.

The present invention relates to photographic materials, and to a method of photographic development. More particularly, the present invention relates to developer-incorporated photographic materials and to a method of processing and using the same.

In the usual process of photographic development, the exposed photographic element comprising a support having at least one gelatin silver halide emulsion layer thereon, is immersed in a developing bath containing a silver halide photographic developing agent. The developing bath is normally maintained as a separate processing bath and with continuous use, the bath usually becomes less efficient so that special techniques and replenishments are normally required to maintain optimum processing efficiency. The developing baths of the prior art normally contain a developing agent, a preservative, such as sodium sulfite, and alkali to activate the developing agent, and may also contain other materials, such as sodium bromide (restrainer), antifoggants, etc. The present invention relates to a method of eliminating the usual type of developing bath, and quite unexpectedly obtains optimum results by incorporating certain photographic developing agent-precursors in emulsion layers, or in adjacent layers. The active developing agent is released by alkaline treatment of the layers after exposure.

It is, therefore, an object of the present invention to provide certain developing agent-precursor substances for incorporation in silver halide photographic emulsion layers, or layers adjacent thereto. Another object is to provide silver halide photographic materials which have said precursor substances incorporated in said emulsion layers, or layers adjacent thereto. A further object is to provide processing solutions for the "development" of said emulsion layers. Still another object is to provide a method of processing the emulsion layers of the invention.

The above objects are accomplished by incorporating certain amide compounds in silver halide emulsion layers, or in layers contiguous thereto and, after photographic exposure, treating such layers with an alkaline solution, such as aqueous sodium carbonate, to release active developing agent. The amide compounds of our invention comprise an N-acyl derivative of an aminophenol, preferably a p-aminophenol. The benzene ring of the aminophenol compounds can contain any non-desensitizing conventional substituents ( $R_2$ ), such as alkyl (e.g., methyl, ethyl, t-butyl, n-hexyl, n-octyl, etc.), halogen (e.g., chlorine, bromine, etc.), alkoxy (e.g., methoxy, ethoxy, etc.), acylamido (e.g., acetamido, chloroacetamido, trifluoroacetamido, bromoacetamido, etc.), acyloxy (e.g., acetoxy, chloroacetoxy, trifluoroacetoxy), etc. Typical amide compounds of our invention include for example:

(I)



2

wherein  $R$  represents an alkyl group (for example, an alkyl group containing from about 1 to 3 carbon atoms, such as methyl, ethyl, propyl, etc.), or a halogenoalkyl group (for example, a halogenoalkyl group containing from about 1 to 3 carbon atoms, such as chloromethyl, dichloromethyl, trichloromethyl,  $\beta$ -chloroethyl,  $\beta$ -dichloroethyl,  $\beta$ -trichloroethyl, bromomethyl, fluoromethyl, difluoromethyl, trifluoromethyl, etc.),  $R_1$  represents a hydrogen atom or a lower alkyl group, such as methyl, ethyl, propyl, etc. (especially an alkyl group containing from about 1 to 3 carbon atoms), and  $R_2$  represents one or more substituents, such as those enumerated above.

The developer precursor compounds of our invention can be incorporated in an ordinary photographic silver halide emulsion, or colloidal dispersion of a water-permeable hydrophilic colloid suitable for preparing an undercoat or an overcoat for such silver halide emulsion, by mixing a solution or dispersion of the precursor compound with the silver halide emulsion, or dispersion of hydrophilic colloid, prior to coating. For example, a developer precursor can be made up as an oil dispersion by stirring a solution of 10 grams of the developing agent precursor into 40 grams of warm tricresylphosphate, and then mixing this solution with 100 grams of a 10 percent aqueous gelatin solution containing 10 cc. of a 5 percent aqueous solution of an alkylnaphthylene sodium sulfonate wetting agent. The resulting dispersion can then be homogenized by passing for 5 times through a colloid mill to produce a homogeneous colloid dispersion. Solvents other than tricresylphosphate can be employed, including any of the crystalloidal compounds described in Jelley and Vittum U.S. Patent 2,322,027, issued June 15, 1943. The resulting colloidal dispersion can then be added to an ordinary silver halide emulsion, or a dispersion of a water-permeable hydrophilic colloid, adapted for preparation of an undercoat or overcoat for such silver halide emulsion.

Instead of adding the oil dispersion directly to the liquid silver halide emulsion or colloidal dispersion, it can be dried for storage purposes and then be reconstituted for use by merely mixing with water.

The developing agent precursors of our invention can be adapted for addition to a liquid silver halide emulsion or colloidal dispersion by other means as well. Suitable methods will depend largely upon the solubility characteristics, particularly in water or polar solvents, of the particular precursors in question. For example, a 1:1 aqueous methanol solution of p-hydroxyacetanilide can be prepared easily, while less water-soluble material can be dissolved or dispersed more easily in a phenolic solvent, or as an oil dispersion as described above.

After addition of the dispersion or solution of the developing agent precursor substance to the liquid emulsion or colloidal dispersion, the mixture is stirred to assure uniform results, or passed through a blending device, such as a colloid mill or Waring Blender. A uniform coating can then be made on a suitable support and the coating dried. Suitable supports comprise any of the well known supporting materials, such as cellulose ester film base (e.g., cellulose acetate, cellulose nitrate, cellulose acetate butyrate, cellulose acetate propionate, etc.), polyethylene, polypropylene, polystyrene, polyethylene terephthalate and other polyesters, paper, polycarbonates, etc.

The photographic elements of our invention comprising a photographic development precursor either in the photographic silver halide emulsion layer, or layer contiguous thereto, or both, can then be exposed to an original or negative and developed by merely treating the exposed emulsion layer with an alkaline activator bath. Typical

activator baths comprise, for example, an aqueous solution of an alkaline material, such as sodium carbonate, sodium hydroxide, potassium carbonate, potassium hydroxide, mixtures of sodium hydroxide and sodium sulfite, etc. Suitable baths can comprise, for example an aqueous solution containing about 1 percent sodium hydroxide and 5 percent sodium sulfite. A bath of the latter type is quite suitable for developing an exposed emulsion layer in about 30 seconds when the activator bath is at about 68° F. Modifications can easily be made in the activator baths without departing from the spirit and scope of the invention. For example, an aqueous solution comprising about 4 percent of sodium carbonate and 5 percent of sodium sulfite produces development in about 30 seconds at 68° F. Another aqueous activator solution comprising 2 percent sodium hydroxide and 5 percent sodium sulfite produces useful photographic images in a few seconds when heated at 130° F. Particularly useful activator solutions have a pH of at least about 9.0 and preferably of at least about 10.5.

The activator solutions of the present invention can be applied to an exposed photographic element in any number of known ways, such as by dipping, spraying, or other suitable surface applications. If desired, a thickener can be added to the activator solution to increase the viscosity of the composition and make it more adaptable for continuous processing. Viscous compositions can then be removed by squeegeeing or water spraying. The photographic element can then be stabilized by conventional fixation or stabilization, such as by sodium thiosulfate.

The concentration of the amide compounds used in our invention will vary, depending upon the particular chemical compound involved and the location of the compound within the photographic element. That is, if the amide compound is incorporated within the silver halide emulsion undergoing development, it may be desirable to use a somewhat different concentration than would be used if the amide compound were incorporated in a layer contiguous to the photographic silver halide emulsion. A useful concentration of amide compound for incorporation in the emulsion is from about 0.1 to 4.0 moles per mole of silver halide. A particularly useful range is from about 0.25 to 2.0 moles per mole of silver halide, with especially useful results being obtained within the range of about 0.4 to 1.0 mole per mole of silver halide. For incorporation in layer contiguous to the silver halide emulsion layer, somewhat larger concentrations of amide compound can be tolerated without adverse effects. A particularly useful effect of our invention is that even when incorporated within the silver halide emulsion, the amide compounds of Formula I have little or no desensitizing effects. In many cases, this is not true where developing agents, *per se*, are incorporated within the silver halide emulsion layers.

Photographic silver halide emulsions useful in our invention comprise any of the ordinarily employed silver halide developing out emulsions, such as, silver-chloride, -chlorobromide, chloroiodide, -chlorobromoiodide, -bromide and -bromoiodide developing-out emulsions. Any of the conventionally employed water-permeable hydrophilic colloids can be employed in the silver halide emulsions, or in layer contiguous thereto. Typical water-permeable hydrophilic colloids include gelatin, albumin, polyvinyl alcohol, agar agar, sodium alginate, hydrolyzed cellulose esters, hydrophilic polyvinyl copolymers, etc.

Photographic silver halide emulsion useful in our invention can also contain such addenda as chemical sensitizers, e.g., sulfur sensitizers (e.g., allyl thiocarbamate, thiourea, allyl isothiocyanate, cystine, etc.), various gold compounds (e.g., potassium chloroaurate, auric trichloride, etc.). (See U.S. Patents 2,540,085, 2,597,856 and 2,597,915, etc.)

Photographic silver halide emulsions useful in our invention can also be sensitized by other means, such as by alkylene oxide polymers, many of which are well known

to those skilled in the photographic art. Typical polyalkylene oxide polymers include those of U.S. Patents 2,423,549 and 2,441,389.

The emulsions of the invention can also contain speed-increasing compounds of the quaternary ammonium type as described in U.S. Patents 2,271,623, issued February 3, 1942; 2,288,226, issued June 30, 1942; 2,334,864, issued November 23, 1943; or the thiopolymers as described in Graham et al. U.S. Patent No. 3,046,129, issued July 24, 1962, and Dann et al. U.S. Patent 3,046,134, issued July 24, 1962.

The emulsions may also be chemically sensitized with reducing agents such as stannous salts (Carroll U.S. Patent 2,487,850), polyamines such as diethylenetriamine (Lowe and Jones U.S. Patent 2,518,698), polyamines such as spermine (Lowe and Allen U.S. Patent 2,521,925), or bis-( $\beta$ -aminoethyl) sulfide and its water-soluble salts (Lowe and Jones U.S. Patent 2,521,926).

The emulsions may also be stabilized with the mercury compounds of Allen, Byers and Murray U.S. application Serial No. 319,611; Carroll and Murray U.S. application Serial No. 319,612; and Leubner and Murray U.S. application Serial No. 319,613, all filed November 8, 1952, now U.S. Patents 2,728,663, 2,728,664 and 2,728,665, respectively, granted December 27, 1955.

The addenda which we have described may be used in various kinds of photographic emulsions. In addition to being useful in X-ray and other nonoptically sensitized emulsions, they may also be used in orthochromatic, panchromatic, and infrared sensitive emulsions. They may be added to the emulsion before or after any sensitizing dyes which are used. The agents may be used in emulsions intended for color photography, for example, emulsions containing color-forming couplers or emulsions to be developed by solutions containing couplers or other color-generating materials, emulsions of the mixed-packet type, such as described in Godowsky U.S. Patent 2,698-794, issued January 9, 1955; or emulsions of the mixed-grain type, such as described in Carroll and Hanson U.S. Patent 2,592,243.

It has been found that the development rate of the compounds represented by Formula I above sometimes can be improved by adding an auxiliary developing agent either to the silver halide emulsion layer, or a hydrophilic layer contiguous thereto. Typical auxiliary developing agents include those described in Belgian Patent 621,608, issued September 14, 1962, of P. H. Stewart, G. E. Falleisen and J. W. Reeves, Jr. Typical auxiliary developing agents described in this patent include 3-pyrazolidone compounds containing an alkyl (e.g., methyl, ethyl, etc.) or aryl substituent (e.g., phenyl, *p*-tolyl, etc.). In addition, such pyrazolidone developing agents can contain an acyl or acyloxy substituent which can be hydrolyzed from the 3-pyrazolidone compound by treatment with the above activator solutions to produce the desired auxiliary developing compound. Typical auxiliary developing agents include, for example,

1-phenyl-3-pyrazolidone,  
1-*p*-tolyl-3-pyrazolidone,  
1-phenyl-3-methyl-3-pyrazolidone,  
1-acetamidophenyl-3-pyrazolidone,  
3-acetoxy-1-phenyl-3-pyrazolidone (Enol ester),  
2-(pyridinium acetyl)-1-phenyl-3-pyrazolidone chloride,  
1-phenyl-4,4-dimethyl-3-pyrazolidone,  
1-phenyl-4-methyl-3-pyrazolidone,  
1-phenyl-2-benzoyl-3-pyrazolidone,  
1-phenyl-2-lauroyl-3-pyrazolidone,  
1-phenyl-2-chloroacetyl-3-pyrazolidone, etc.

The concentration of auxiliary developing agents can be varied and, of course, no auxiliary developing agent need be employed unless so desired. Useful concentrations of auxiliary developing agents vary from about 0.01 mole to 2.0 moles per mole of amide compound. De-

pending upon the particular auxiliary developing agent employed, larger or smaller quantities can be used.

It has also been found that the development precursors of our invention can be used quite effectively with a development precursor of the hydroquinone type, such as those described in our copending applications Serial Nos. 183,354, filed March 29, 1962, now abandoned, and 366,127, filed May 8, 1964, now U.S. Patent No. 3,246,988. The hydroquinone type of development precursor includes those wherein one or both of the phenolic hydroxyl radicals has been esterified with an organic acid, anhydride or halide, as described in such applications. The esterification can be accomplished by means which have already been described in the prior art, where a reaction mixture containing both hydroquinone compound and organic acid, anhydride or halide is heated, preferably in the presence of a basic condensation agent. The resulting mono- or di-esters can then be used together with the amide development precursors of this application. In general, the quantity of development precursor of the hydroquinone type can be from about 10 to about 200 mole percent of the quantity of amide precursor. The hydroquinone type of development precursor can be incorporated in the photographic elements of our invention in the manner described below. Organic acids which can be used as such, or in the form of their anhydrides or halides, to esterify the hydroquinone compound include acids, such as acetic, propionic, butyric, etc., which may have one or more halogen substituents on the carbon atoms of such acids. Typical halogen substituents include chlorine, bromine and fluorine, for example.

The amide derivatives of Formula I above can easily be prepared by reacting an organic acid, an anhydride or halide with the corresponding aminophenol compound (nuclear substituted or unsubstituted).

The following examples will serve to illustrate the preparation of typical amide compounds or intermediates.

#### Example 1

p-(N-methyl-N-trifluoroacetyl)aminophenol for incorporating in a silver halide emulsion layer according to the invention was prepared by adding 14 g. of p-methylaminophenol to 100 ml. of trifluoroacetic anhydride resulting in an exothermic reaction and forming a dark solution which was maintained at reflux for about two and a half days. The solvent was evaporated from the solution yielding a heavy oil that was triturated with 100 ml. of cold water. The resultant oil was air dried to produce a crystalline solid having a melting point of 109-111° C. and was crystallized from chloroform-ligroin to yield 17.21 g. of pinkish-white prisms having a melting point of 103-104° C.

Analytical calculation for  $C_9H_8O_2NF_3$ : C, 49.4; H, 3.68; N, 6.40. Found: C, 49.2; H, 3.8; N, 6.6, 6.7.

#### Example 2

p-(N-trifluoroacetyl)aminophenol suitable for use as an incorporated developer precursor according to the present invention was prepared by adding 250 g. of trifluoroacetic anhydride dropwise into a vessel containing 54.6 g. p-aminophenol after which the mixture was stirred and maintained at 5° C. and refluxed continuously overnight. After cooling, the solution was poured into 750 ml. of ice water to give a brown oil. The aqueous phase was decanted, the oil washed rapidly with warm water and subsequently evaporated to dryness with 500 ml. of benzene. The oil was crystallized from acetone-benzene and recrystallized from chloroform several times to give 12.72 g. of white flakes having a melting point of 173.5-174° C.

Analytical calculation for  $C_8H_6O_2NF_3$ : C, 46.9; H, 2.95; N, 6.83. Found: C, 47.0; H, 3.2; N, 7.2.

Other amide types of development precursors can be prepared in a manner similar to that illustrated in Examples 1 and 2 above, as well as by techniques which have been described in the prior art. For example, p-hydroxy-

acetanilide which is a useful development precursor in our invention can be prepared as described in Beilstein, vol. 13, page 460. In a similar manner, p-hydroxy- $\omega$ -chloroacetanilide can be prepared as described in Beilstein, vol. 13, first supplement, page 160. In a like manner, other substituted derivatives of aminophenols can be prepared using a mixture of free amine and acylating agent, such as those illustrated above.

The following examples will serve to illustrate the useful effects of our development precursors when incorporated within an ordinary photographic silver halide emulsion.

#### Example 3

In a manner described above, a number of oil dispersions in tricresylphosphate (10 grams of developing agent precursors in 40 grams of tricresylphosphate) were prepared. A "blank" dispersion (no developer precursor) was prepared in an identical manner to serve as a control. These dispersions were separately added to aliquot portions of an ordinary photographic gelatino-silver-bromide emulsion in the concentrations shown in the following table. The developing agent precursors are identified according to preparative example number. The table below also illustrates the useful effect obtained when a small amount of a developing agent, per se, was added to certain of the aliquot portions. These developing agents were added to the emulsions from an alcohol solution. The treated emulsion samples were separately coated on cellulose acetate supports, dried and exposed to tungsten illumination on an Eastman Type Ib Sensitometer. The coatings were then developed by treatment with an alkaline activator solution containing 1% sodium hydroxide and 5% sodium sulfite, development being effective by immersion for 15 seconds at 100° F. The relative speed for each of the coatings was measured at a point 0.3 above fog in the usual manner. The following results were obtained.

TABLE A

| Coating | Addenda—Compound of Example                                           | Rel. Speed | $\gamma$ | $D_{max.}$ |
|---------|-----------------------------------------------------------------------|------------|----------|------------|
| A-1.    | None—control                                                          | Nil        | Nil      | Nil        |
| A-2.    | p-Acetoxyphenol (0.5 mole)                                            | 100        | .49      | 1.4        |
| A-3.    | p-Acetoxyphenol (0.5 mole) plus N-methyl-p-aminophenol sulfate (4 g.) | 100        | 0.55     | 1.5        |
| A-4.    | p-Acetoxyphenol (0.5 mole) plus 1 (5.1 g.)                            | 150        | 0.80     | 1.9        |

#### Example 4

Several gelatin dispersions were prepared according to the technique described in Example 3 using warm tricresylphosphate as a solvent for the development agent precursors identified in the following table. As in Example 3, a "blank" dispersion containing no development agent precursor was prepared to serve as a control. In addition, a number of compounds corresponding to the amide compounds illustrated were added to similar portions of emulsion in order to show the effect of acylation on the amino radical of such compounds.

The dispersions of development precursors or their corresponding free-amines were added to ordinary gelatino-silver-bromide emulsions at the concentration shown in Table B below. The silver halide emulsion used was a conventional gold and sulfur sensitized, high-speed emulsion which had been panchromatically sensitized. The dispersions were then coated on conventional cellulose acetate film support and dried. Each sample was then exposed on an ordinary Eastman Ib Sensitometer and processed in an ordinary alkaline activating bath, such as aqueous sodium carbonate, or an aqueous solution containing 2% sodium hydroxide and 5% sodium sulfite. Treatment was for the time indicated in the table. In addition, strips of such coatings were

developed for 5 minutes in Kodak Developer DK-50, which has the following composition:

|                                |       |      |
|--------------------------------|-------|------|
| Water, about 125° F. (50° C.)  | cc.   | 500  |
| N-methyl-p-aminophenol sulfate | grams | 2.5  |
| Sodium sulfite, desiccated     | do    | 30.0 |
| Hydroquinone                   | do    | 2.5  |
| Sodium metaborate              | do    | 10.0 |
| Potassium bromide              | do    | 0.5  |
| Water to make 1.0 liter.       |       |      |

Each of the film samples was then fixed, washed and dried and the number of 0.2 log E steps read in order to determine the density obtainable with such development precursors. It is obvious from the table that the acylated compounds had a much more useful effect than the unacylated derivatives. In particular, the fog levels were

10  
15  
16  
17  
18  
19  
20  
21  
22  
23  
24  
25  
26  
27  
28  
29  
30  
31  
32  
33  
34  
35  
36  
37  
38  
39  
40  
41  
42  
43  
44  
45  
46  
47  
48  
49  
50  
51  
52  
53  
54  
55  
56  
57  
58  
59  
60  
61  
62  
63  
64  
65  
66  
67  
68  
69  
70  
71  
72  
73  
74  
75  
76  
77  
78  
79  
80  
81  
82  
83  
84  
85  
86  
87  
88  
89  
90  
91  
92  
93  
94  
95  
96  
97  
98  
99  
100  
101  
102  
103  
104  
105  
106  
107  
108  
109  
110  
111  
112  
113  
114  
115  
116  
117  
118  
119  
120  
121  
122  
123  
124  
125  
126  
127  
128  
129  
130  
131  
132  
133  
134  
135  
136  
137  
138  
139  
140  
141  
142  
143  
144  
145  
146  
147  
148  
149  
150  
151  
152  
153  
154  
155  
156  
157  
158  
159  
160  
161  
162  
163  
164  
165  
166  
167  
168  
169  
170  
171  
172  
173  
174  
175  
176  
177  
178  
179  
180  
181  
182  
183  
184  
185  
186  
187  
188  
189  
190  
191  
192  
193  
194  
195  
196  
197  
198  
199  
200  
201  
202  
203  
204  
205  
206  
207  
208  
209  
210  
211  
212  
213  
214  
215  
216  
217  
218  
219  
220  
221  
222  
223  
224  
225  
226  
227  
228  
229  
230  
231  
232  
233  
234  
235  
236  
237  
238  
239  
240  
241  
242  
243  
244  
245  
246  
247  
248  
249  
250  
251  
252  
253  
254  
255  
256  
257  
258  
259  
260  
261  
262  
263  
264  
265  
266  
267  
268  
269  
270  
271  
272  
273  
274  
275  
276  
277  
278  
279  
280  
281  
282  
283  
284  
285  
286  
287  
288  
289  
290  
291  
292  
293  
294  
295  
296  
297  
298  
299  
300  
301  
302  
303  
304  
305  
306  
307  
308  
309  
310  
311  
312  
313  
314  
315  
316  
317  
318  
319  
320  
321  
322  
323  
324  
325  
326  
327  
328  
329  
330  
331  
332  
333  
334  
335  
336  
337  
338  
339  
340  
341  
342  
343  
344  
345  
346  
347  
348  
349  
350  
351  
352  
353  
354  
355  
356  
357  
358  
359  
360  
361  
362  
363  
364  
365  
366  
367  
368  
369  
370  
371  
372  
373  
374  
375  
376  
377  
378  
379  
380  
381  
382  
383  
384  
385  
386  
387  
388  
389  
390  
391  
392  
393  
394  
395  
396  
397  
398  
399  
400  
401  
402  
403  
404  
405  
406  
407  
408  
409  
410  
411  
412  
413  
414  
415  
416  
417  
418  
419  
420  
421  
422  
423  
424  
425  
426  
427  
428  
429  
430  
431  
432  
433  
434  
435  
436  
437  
438  
439  
440  
441  
442  
443  
444  
445  
446  
447  
448  
449  
450  
451  
452  
453  
454  
455  
456  
457  
458  
459  
460  
461  
462  
463  
464  
465  
466  
467  
468  
469  
470  
471  
472  
473  
474  
475  
476  
477  
478  
479  
480  
481  
482  
483  
484  
485  
486  
487  
488  
489  
490  
491  
492  
493  
494  
495  
496  
497  
498  
499  
500  
501  
502  
503  
504  
505  
506  
507  
508  
509  
510  
511  
512  
513  
514  
515  
516  
517  
518  
519  
520  
521  
522  
523  
524  
525  
526  
527  
528  
529  
530  
531  
532  
533  
534  
535  
536  
537  
538  
539  
540  
541  
542  
543  
544  
545  
546  
547  
548  
549  
550  
551  
552  
553  
554  
555  
556  
557  
558  
559  
5510  
5511  
5512  
5513  
5514  
5515  
5516  
5517  
5518  
5519  
5520  
5521  
5522  
5523  
5524  
5525  
5526  
5527  
5528  
5529  
55210  
55211  
55212  
55213  
55214  
55215  
55216  
55217  
55218  
55219  
55220  
55221  
55222  
55223  
55224  
55225  
55226  
55227  
55228  
55229  
55230  
55231  
55232  
55233  
55234  
55235  
55236  
55237  
55238  
55239  
55240  
55241  
55242  
55243  
55244  
55245  
55246  
55247  
55248  
55249  
55250  
55251  
55252  
55253  
55254  
55255  
55256  
55257  
55258  
55259  
55260  
55261  
55262  
55263  
55264  
55265  
55266  
55267  
55268  
55269  
55270  
55271  
55272  
55273  
55274  
55275  
55276  
55277  
55278  
55279  
55280  
55281  
55282  
55283  
55284  
55285  
55286  
55287  
55288  
55289  
55290  
55291  
55292  
55293  
55294  
55295  
55296  
55297  
55298  
55299  
552100  
552101  
552102  
552103  
552104  
552105  
552106  
552107  
552108  
552109  
552110  
552111  
552112  
552113  
552114  
552115  
552116  
552117  
552118  
552119  
552120  
552121  
552122  
552123  
552124  
552125  
552126  
552127  
552128  
552129  
552130  
552131  
552132  
552133  
552134  
552135  
552136  
552137  
552138  
552139  
552140  
552141  
552142  
552143  
552144  
552145  
552146  
552147  
552148  
552149  
552150  
552151  
552152  
552153  
552154  
552155  
552156  
552157  
552158  
552159  
552160  
552161  
552162  
552163  
552164  
552165  
552166  
552167  
552168  
552169  
552170  
552171  
552172  
552173  
552174  
552175  
552176  
552177  
552178  
552179  
552180  
552181  
552182  
552183  
552184  
552185  
552186  
552187  
552188  
552189  
552190  
552191  
552192  
552193  
552194  
552195  
552196  
552197  
552198  
552199  
552200  
552201  
552202  
552203  
552204  
552205  
552206  
552207  
552208  
552209  
552210  
552211  
552212  
552213  
552214  
552215  
552216  
552217  
552218  
552219  
552220  
552221  
552222  
552223  
552224  
552225  
552226  
552227  
552228  
552229  
5522210  
5522211  
5522212  
5522213  
5522214  
5522215  
5522216  
5522217  
5522218  
5522219  
5522220  
5522221  
5522222  
5522223  
5522224  
5522225  
5522226  
5522227  
5522228  
5522229  
55222210  
55222211  
55222212  
55222213  
55222214  
55222215  
55222216  
55222217  
55222218  
55222219  
55222220  
55222221  
55222222  
55222223  
55222224  
55222225  
55222226  
55222227  
55222228  
55222229  
55222210  
55222211  
55222212  
55222213  
55222214  
55222215  
55222216  
55222217  
55222218  
55222219  
55222220  
55222221  
55222222  
55222223  
55222224  
55222225  
55222226  
55222227  
55222228  
55222229  
55222210  
55222211  
55222212  
55222213  
55222214  
55222215  
55222216  
55222217  
55222218  
55222219  
55222220  
55222221  
55222222  
55222223  
55222224  
55222225  
55222226  
55222227  
55222228  
55222229  
55222210  
55222211  
55222212  
55222213  
55222214  
55222215  
55222216  
55222217  
55222218  
55222219  
55222220  
55222221  
55222222  
55222223  
55222224  
55222225  
55222226  
55222227  
55222228  
55222229  
55222210  
55222211  
55222212  
55222213  
55222214  
55222215  
55222216  
55222217  
55222218  
55222219  
55222220  
55222221  
55222222  
55222223  
55222224  
55222225  
55222226  
55222227  
55222228  
55222229  
55222210  
55222211  
55222212  
55222213  
55222214  
55222215  
55222216  
55222217  
55222218  
55222219  
55222220  
55222221  
55222222  
55222223  
55222224  
55222225  
55222226  
55222227  
55222228  
55222229  
55222210  
55222211  
55222212  
55222213  
55222214  
55222215  
55222216  
55222217  
55222218  
55222219  
55222220  
55222221  
55222222  
55222223  
55222224  
55222225  
55222226  
55222227  
55222228  
55222229  
55222210  
55222211  
55222212  
55222213  
55222214  
55222215  
55222216  
55222217  
55222218  
55222219  
55222220  
55222221  
55222222  
55222223  
55222224  
55222225  
55222226  
55222227  
55222228  
55222229  
55222210  
55222211  
55222212  
55222213  
55222214  
55222215  
55222216  
55222217  
55222218  
55222219  
55222220  
55222221  
55222222  
55222223  
55222224  
55222225  
55222226  
55222227  
55222228  
55222229  
55222210  
55222211  
55222212  
55222213  
55222214  
55222215  
55222216  
55222217  
55222218  
55222219  
55222220  
55222221  
55222222  
55222223  
55222224  
55222225  
55222226  
55222227  
55222228  
55222229  
55222210  
55222211  
55222212  
55222213  
55222214  
55222215  
55222216  
55222217  
55222218  
55222219  
55222220  
55222221  
55222222  
55222223  
55222224  
55222225  
55222226  
55222227  
55222228  
55222229  
55222210  
55222211  
55222212  
55222213  
55222214  
55222215  
55222216  
55222217  
55222218  
55222219  
55222220  
55222221  
55222222  
55222223  
55222224  
55222225  
55222226  
55222227  
55222228  
55222229  
55222210  
55222211  
55222212  
55222213  
55222214  
55222215  
55222216  
55222217  
55222218  
55222219  
55222220  
55222221  
55222222  
55222223  
55222224  
55222225  
55222226  
55222227  
55222228  
55222229  
55222210  
55222211  
55222212  
55222213  
55222214  
55222215  
55222216  
55222217  
55222218  
55222219  
55222220  
55222221  
55222222  
55222223  
55222224  
55222225  
55222226  
55222227  
55222228  
55222229  
55222210  
55222211  
55222212  
55222213  
55222214  
55222215  
55222216  
55222217  
55222218  
55222219  
55222220  
55222221  
55222222  
55222223  
55222224  
55222225  
55222226  
55222227  
55222228  
55222229  
55222210  
55222211  
55222212  
55222213  
55222214  
55222215  
55222216  
55222217  
55222218  
55222219  
55222220  
55222221  
55222222  
55222223  
55222224  
55222225  
55222226  
55222227  
55222228  
55222229  
55222210  
55222211  
55222212  
55222213  
55222214  
55222215  
55222216  
55222217  
55222218  
55222219  
55222220  
55222221  
55222222  
55222223  
55222224  
55222225  
55222226  
55222227  
55222228  
55222229  
55222210  
55222211  
55222212  
55222213  
55222214  
55222215  
55222216  
55222217  
55222218  
55222219  
55222220  
55222221  
55222222  
55222223  
55222224  
55222225  
55222226  
55222227  
55222228  
55222229  
55222210  
55222211  
55222212  
55222213  
55222214  
55222215  
55222216  
55222217  
55222218  
55222219  
55222220  
55222221  
55222222  
55222223  
55222224  
55222225  
55222226  
55222227  
55222228  
55222229  
55222210  
55222211  
55222212  
55222213  
55222214  
55222215  
55222216  
55222217  
55222218  
55222219  
55222220  
55222221  
55222222  
55222223  
55222224  
55222225  
55222226  
55222227  
55222228  
55222229  
55222210  
55222211  
55222212  
55222213  
55222214  
55222215  
55222216  
55222217  
55222218  
55222219  
55222220  
55222221  
55222222  
55222223  
55222224  
55222225  
55222226  
55222227  
55222228  
55222229  
55222210  
55222211  
55222212  
55222213  
55222214  
55222215  
55222216  
55222217  
55222218  
55222219  
55222220  
55222221  
55222222  
55222223  
55222224  
55222225  
55222226  
55222227  
55222228  
55222229  
55222210  
55222211  
55222212  
55222213  
55222214  
55222215  
55222216  
55222217  
55222218  
55222219  
55222220  
55222221  
55222222  
55222223  
55222224  
55222225  
55222226  
55222227  
55222228  
55222229  
55222210  
55222211  
55222212  
55222213  
55222214  
55222215  
55222216  
55222217  
55222218  
55222219  
55222220  
55222221  
55222222  
55222223  
55222224  
55222225  
55222226  
55222227  
55222228  
55222229  
55222210  
55222211  
55222212  
55222213  
55222214  
55222215  
55222216  
55222217  
55222218  
55222219  
55222220  
55222221  
55222222  
55222223  
55222224  
55222225  
55222226  
55222227  
55222228  
55222229  
55222210  
55222211  
55222212  
55222213  
55222214  
55222215  
55222216  
55222217  
55222218  
55222219  
55222220  
55222221  
55222222  
55222223  
55222224  
55222225  
55222226  
55222227  
55222228  
55222229  
55222210  
55222211  
55222212  
55222213  
55222214  
55222215  
55222216  
55222217  
55222218  
55222219  
55222220  
55222221  
55222222  
55222223  
55222224  
55222225  
55222226  
55222227  
55222228  
55222229  
55222210  
55222211  
55222212  
55222213  
55222214  
55222215  
55222216  
55222217  
55222218  
55222219  
55222220  
55222221  
55222222  
55222223  
55222224  
55222225  
55222226  
55222227  
55222228  
55222229  
55222210  
55222211  
55222212  
55222213  
55222214  
55222215  
55222216  
55222217  
55222218  
55222219  
55222220  
55222221  
55222222  
55222223  
55222224  
55222225  
55222226  
55222227  
55222228  
55222229  
55222210  
55222211  
55222212  
55222213  
55222214  
55222215  
55222216  
55222217  
55222218  
55222219  
55222220  
55222221  
55222222  
55222223  
55222224  
55222225  
55222226  
55222227  
55222228  
55222229  
55222210  
55222211  
55222212  
55222213  
55222214  
55222215<br

such as described in Haist et al. U.S. Patent 2,875,048, issued February 24, 1959, and in web-type processes, such as the one described in Tregillus et al. U.S. patent application Serial No. 835,473, filed August 24, 1959, now U.S. Patent No. 3,179,517.

Of course, the activator solutions which are used in our invention are stable for extended periods of time and are not subject to the harmful decomposition reactions so common to conventional photographic developing solutions when these developing solutions are stored for extended periods of time. No special precautions are required to prevent oxidation of the activator solutions since they are inherently quite stable. If desired, the activator solutions can be incorporated in a carrier, such as gelatin and coated in contact with the photographic silver halide emulsion layer which contains the development precursors of our invention. After exposure, the development can be effected merely by heating the photographic emulsion layer to a temperature sufficient to release water, which may be present in the support or in a separate layer in the photographic element. This water then dissolves the activator solution from the hydrophilic colloid layers and takes it into the photographic halide emulsion layer where the emulsion is effected.

The elevated temperatures from about 95-150° C. are usually sufficient to effect development in this manner. If desired, additional moisture can be added by spraying steam upon the sensitive surface of the photographic element.

The invention has been described in detail with particular reference to preferred embodiments thereof, but it will be understood that variations and modifications can be effected within the spirit and scope of the invention as described hereinabove and as defined in the appended claims.

We claim:

1. A photographic element comprising a support and a photographic silver halide emulsion layer, and integral with said photographic element a water-permeable, hydrophilic colloid containing a silver halide development precursor represented by the following general formula:



wherein R represents a member selected from the class consisting of an alkyl group and a halogenoalkyl group, R<sub>1</sub> represents a member selected from the class consisting of a hydrogen atom and an alkyl group, and R<sub>2</sub> represents a member selected from the class consisting of a hydrogen atom, an alkyl group, a halogen atom, an alkoxy group, an acylamido group and an acyloxy group.

2. A photographic element as defined in claim 1 wherein said precursor is incorporated in said silver halide emulsion layer.

3. A photographic element as defined in claim 1 wherein said precursor is incorporated in a hydrophilic colloid layer contiguous to said silver halide emulsion layer.

4. A photographic element as defined in claim 1 wherein said precursor is incorporated in said photographic element as a dispersion in a water-insoluble, crystalloidal solvent.

5. A photographic element as defined in claim 1 wherein said precursor is o-(N-trifluoroacetyl)aminophenol.

6. A photographic element as defined in claim 1

wherein said precursor is p-(N-trifluoroacetyl)aminophenol.

7. A photographic element as defined in claim 1 wherein said precursor is p-(N-methyl-N-trifluoroacetyl)aminophenol.

8. A photographic element as defined in claim 1 wherein said precursor is m-methyl-p-(N-trifluoroacetyl)aminophenol.

9. A photographic element as defined in claim 1 wherein said precursor is 2,4-(N,N-trifluoroacetyl)diaminophenol.

10. A photographic element comprising a support and a photographic silver halide emulsion layer, and integral with said photographic element a water-permeable, hydrophilic colloid containing a development precursor represented by the following general formula:



wherein R represents a member selected from the class consisting of an alkyl group and a halogenoalkyl group, R<sub>1</sub> represents a member selected from the class consisting of a hydrogen atom and an alkyl group, and R<sub>2</sub> represents a member selected from the class consisting of a hydrogen atom, an alkyl group, a halogen atom, an alkoxy group, an acylamido group and an acyloxy group, said photographic element containing in addition to said development precursor a 3-pyrazolidone photographic silver halide developing agent.

11. A photographic element comprising a support and a photographic silver halide emulsion layer, and integral with said photographic element a water-permeable, hydrophilic colloid containing a development precursor represented by the following general formula:



wherein R represents a member selected from the class consisting of an alkyl group and a halogenoalkyl group, R<sub>1</sub> represents a member selected from the class consisting of a hydrogen atom and an alkyl group, and R<sub>2</sub> represents a member selected from the class consisting of a hydrogen atom, an alkyl group, a halogen atom, an alkoxy group, an acylamido group and an acyloxy group, said photographic element containing in addition to said development precursor a hydroquinone silver halide developing agent precursor, at least one of whose hydroxyl radicals has been esterified to form an ester hydrolyzable in aqueous alkaline solution.

#### References Cited by the Examiner

#### UNITED STATES PATENTS

|           |         |                  |         |
|-----------|---------|------------------|---------|
| 1,497,252 | 6/1924  | Theimer          | 260-562 |
| 1,853,455 | 4/1932  | Reddelien et al. | 96-66   |
| 2,653,158 | 9/1953  | Young et al.     | 260-562 |
| 2,751,295 | 6/1956  | Salminen et al.  | 96-95   |
| 3,113,026 | 12/1963 | Sprung           | 96-66   |

NORMAN G. TORCHIN, Primary Examiner,

J. TRAVIS BROWN, Examiner,